

Aug. 7, 1923.

1,464.488

**F. S. BESSON**

## METHOD FOR MAKING BITUMINOUS PAVING MIXTURES

Filed May 26, 1921



Frank S. Sessions

## UNITED STATES PATENT OFFICE.

FRANK S. BESSON, OF WASHINGTON, DISTRICT OF COLUMBIA.

## METHOD FOR MAKING BITUMINOUS PAVING MIXTURES.

Application filed May 26, 1921. Serial No. 472,889.

(FILED UNDER THE ACT OF MARCH 3, 1883, 22 STAT. L., 625.)

*To all whom it may concern:*

Be it known that I, FRANK S. BESSON, a citizen of the United States, and a resident of Washington, District of Columbia, have 5 invented an Improvement in Methods for Making Bituminous Paving Mixtures, of which the following is a specification.

The invention described herein may be used by the Government, or any of its officers 10 or employees in prosecution of work for the Government, or by any other person in the United States, without payment to me of any royalty thereon.

This invention relates to paving mixtures, 15 more particularly to a new and improved method by which the bituminous binding agent and mineral aggregate are correctly proportioned and combined to produce an efficient mixture for highways, sidewalks, 20 floors and similar constructions.

One of the principal purposes of this invention is to provide a formula for paving mixtures, which will afford uniform paving 25 results and permit an accurate determination of the bituminous requirements for any character of mineral aggregate.

Another important object of this invention is to provide a formula which will enable the 30 bitumen requirement for any given quantity of mineral aggregate to be proportioned in accordance with the void percentage and specific gravity of the aggregate.

Another important object of this invention is to produce a paving mixture characterized by its wear resisting qualities and 35 ability to resist deterioration, crawling, creeping, undue deformation or fracture when subjected to traffic wear or adverse moisture and heat conditions.

With these and other objects in view, 40 this invention consists in certain novel combining and proportioning of materials as will be hereinafter more fully set forth and claimed.

In attempting to solve the problem of producing a successful paving mixture, highway engineers have advanced and resorted 45 to many theories and formulas, some advocating "surface area of aggregate", the mechanical analysis, accumulative plat, or fineness modulus methods; while others have attached considerable importance to density measurements of samples taken from streets, or have contended that wavy pavements

originate in the use of sand or mineral aggregate 55 the grains of which are round and smooth instead of angular and rough.

Actual experiments, however, prove the fallacy of these theories, as mixtures made 60 in accordance with the same formulas vary in many respects, one resultant surface being excellent, another corrugated and waved, and still another cracked and disintegrated.

In an endeavor to find a solution to this problem many experiments have been made 65 and the result of these tests indicate that defective pavements are often traceable to an improper proportion of bitumen in the mixture. It is therefore the aim and purpose of this invention to provide a formula 70 which will enable the correct amount of bitumen for any particular aggregate to be accurately determined, and in this connection it is to be understood, that the term "aggregate" as used hereinafter in the description and claims, embraces the total mineral matter of the mixture. 75

In the accompanying drawing, the figure is a graphical representation of the relationship between bitumen requirements, aggregate voidage, specific gravity, and resulting satisfactory paving. 80

Coming now to the subject matter of the present invention, numerous experimental tests with samples of existing pavements 85 have definitely established the following facts:

(a) That sieve analyses of mineral aggregates do not afford an accurate basis for determining bitumen requirements. 90

(b) That specimens of imperfect surfaces prepared by sieve analysis formulae supposedly correct, indicate, according to the defective conditions of the paving, either too much or insufficient bitumen, as required 95 by the void percentage and specific gravity of the aggregate.

(c) That definite relations exist between the bitumen requirements, void percentage, and specific gravity of the aggregate. 100

(d) The proportion by weight of bitumen to aggregate depends upon the volume of a given weight of aggregate.

With the preceding facts established many investigations were made of specimens having a definite volume (one thousand cubic centimeters) taken from Washington thoroughfares, which had rendered satisfactory

service over a number of years; each specimen being analyzed to determine—

(a) Bitumen contents

5 (b) Void percentage and specific gravity of aggregate.

In making these determinations the volume measurements may be made by means of a graduated cylinder 62 millimeters in diameter and of sufficient capacity to hold 10 a thousand grams of material.

After obtaining the bitumen contents of the specimens and the void percentages and specific gravities of the aggregates, a chart is plotted wherein the curve (2) represents 15 the resultant of the abscissas (1) and the ordinates (3) and (4) the specific gravities and bitumen contents expressed in percentages by weight.

With this diagram at hand, to determine 20 the bitumen requirements of an original mixture, the operator determines the void percentage and specific gravity of a thousand grams of dry loose aggregate by any of the usual methods for ascertaining voidage and 25 density of an aggregate, and then with these factors known, consults the chart for the correct amount of bitumen shown by the previously analyzed specimens to be required for an aggregate having a similar void percentage and specific gravity.

To obtain the specific gravity ordinates 30 (3) it is noted that the sloping axes of these ordinates indicate that the bituminous percentages increase inversely as the specific 35 gravity of the aggregates. Thus the vertical axis of ordinates representing percentages for aggregate of specific gravity 3, forms with the 2.3 axis an angle whose cosine is 2.3 divided by 3, and this angle is 40 approximately 40 degrees.

Reference being had to the accompanying drawing, it will be seen that, having ascertained for any particular aggregate the void percentage indicated by ordinates 1, a point 45 may be located on the curve 2, and corresponding to this point on the specific gravity ordinates 3, may be read from ordinates 4 the percentage by weight of bituminous 50 cement testing approximately 99% bitumen soluble in carbon bisulphide, the bitumen being of approximately 1.06 specific gravity.

In order to facilitate estimates, ordinates 55 may be added to and used in conjunction with the diagram for determining the amount of satisfactory pavement resulting per cubic yard of aggregate used.

As a more specific illustration of the application of the accompanying diagram, assuming the percentage of voids to be 41.0 for a 60 given aggregate, having a specific gravity of 2.7; upon entering the diagram with the void percentage of the particular aggregate as an abscissa, a point *a* is located on curve 2 which corresponds to the point *b* on the 65 specific gravity ordinates, thus giving a

reading of 8.2 as the correct percentage of bitumen required for the mixture. In the event ordinates 5 are included in the diagram, a point *c* may be located in this ordinate column which corresponds to the point 70 *a* on curve 2 and gives a reading of approximately 29.2 square yards of pavement 1" thick per cubic yard of aggregate.

In the illustrated embodiment characterizing this invention reference has been made 75 to bituminous cement testing 99% soluble in carbon bisulphide, the bitumen being of approximately 1.06 specific gravity; it is to be understood, however, that the relationship between the void percentage, specific gravity 80 of the mineral matter and amount of bitumen soluble in carbon bisulphide exists irrespective of the character of bituminous cement used, and that proper alteration may readily be made to render the diagram applicable to other bituminous cements, these alterations being made according to the variance in the degree of solubility and specific gravity of the bitumen.

Although in the preceding description a 90 definite method has been outlined for determining the correct amount of bitumen for any particular aggregate dependant on the void percentage and specific gravity of the latter, it is to be understood that other 95 methods may be employed for accomplishing this same result without departing from or sacrificing any of the principles of this invention.

In conclusion, it may be stated that, as this 100 invention by properly proportioning the components of the paving mixture, eliminates waves, cracking, and other unsatisfactory paving results, the binder course ordinarily utilized for overcoming these defects is made unnecessary; in consequence of which a material saving is effected in the cost of concrete constructions of the character under discussion.

Having described my invention, what I 110 claim to be new and wish to protect by Letters Patent is:

A method of making bituminous paving mixtures, consisting in determining the void percentage of a definite volume of a loose aggregate and the specific gravity of the aggregate, with these as factors determining from the graph illustrated in the accompanying drawing the amount of bitumen required for an aggregate having similar void percentage and specific gravity and adding this amount of bitumen to the loose aggregate, such graph being based upon and representing the results of the determinations of the bitumen content, void percentage and specific gravity of a series of selected, differing specimens of satisfactory paving mixtures.

FRANK S. BESSON.